

March 21, 1933.

J. J. VETTER

1,901,939

PROCESS OF PRODUCING CHROMATES

Filed July 3, 1930

2 Sheets-Sheet 1



*Fig. 3.*



*Fig. 4.*

INVENTOR  
Joseph J. Vetter  
BY  
Arthur Wright  
ATTORNEY

March 21, 1933.

J. J. VETTER

1,901,939

PROCESS OF PRODUCING CHROMATES

Filed July 3, 1930

2 Sheets-Sheet 2



## UNITED STATES PATENT OFFICE

JOSEPH J. VETTER, OF HACKENSACK, NEW JERSEY, ASSIGNOR TO NATURAL PRODUCTS  
REFINING CO., OF JERSEY CITY, NEW JERSEY, A CORPORATION OF DELAWARE

## PROCESS OF PRODUCING CHROMATES

Application filed July 3, 1930. Serial No. 465,683.

My invention relates to a process of producing chromates from any suitable materials containing chromium, but relates especially to a treatment of chrome ores such as

capable of being carried out in a great many different types of apparatus, I have shown only certain forms of apparatus for use in connection therewith in the accompanying drawings, in which:

55

Fig. 1 is a diagrammatic representation of an apparatus which may be used in accordance with my invention;

60

Fig. 2 is a vertical section of the kiln used in accordance with my invention;

65

Fig. 3 is a diagrammatic representation of the steps of one form of my invention;

65

Fig. 4 is a diagrammatic representation of the steps in a modified form of my invention; and

70

Fig. 5 is an enlarged cross sectional detail.

Referring to the drawings, I have shown an apparatus comprising an elongated inclined rotary kiln 1, preferably about 10 to 13 times the inside diameter thereof, having any suitable lining 2, and carried upon cylindrical tracks 3 and 4, which are supported upon rollers 5 and 6. The inclined rotary kiln 1 may be driven from any suitable source of power as, for example, by means of a gear 7, carried by the kiln, which meshes with a driving gear 8 connected to any motive power as desired. At its upper end the kiln may be supplied continuously with materials to be treated therein through a hopper 9, having an outlet 10 extending into the kiln. At its lower end there extends into the kiln an elongated burner tube 11 located in an air supply controlling tube 11a provided with a head having air ports 11b movable by a hand wheel 11c screw-threaded thereto and splined in an air tube 11d having a valved air supply 11e extending for a distance of about  $\frac{1}{8}$  to  $\frac{1}{5}$  the length of the kiln, the kiln having a length of about 10 to 18 times the inside diameter thereof. The oil pipe 11 may be supplied with any desired fuel as, for example, gas, but preferably with crude oil which is burned at the inner end of the burner 11 by means of a spray nozzle 12 of any desired type. A pipe 13 of heat resisting steel is located around the burner tube 11 upon a support 13a in such a manner that the outer end thereof draws in a current of air while the inner end of said pipe 13 is so arranged as to permit the escape

75

80

85

90

95

100

5 are used in the manufacture of chromates. The object of my invention is to provide a process of the above character, having many advantages over previous processes used for this purpose. More especially, the object of 10 my invention is to provide a process whereby larger yields of chromates may be obtained and preferably in accordance with a procedure involving lower costs. My process involves, also, the use of a shorter time in the 15 production of products therein. Also, my process may be carried out in such a way, if desired, so as to obviate one of the steps of leaching, thus obviating after the first roasting, the necessity of filtration with its accompanying 20 disadvantages, and consequently obviating the necessity of re-weighing, re-mixing and drying in the course thereof. When carried out in this way, the process may include in the course of the same a grinding 25 operation which enables further oxidation of the partially treated product to be attained, in view of the fact that the lumps formed in the process are broken up, thus presenting new surfaces therein for the action there- 30 on by the materials added.

Hitherto the process for producing chromates from chrome ore necessitated a considerable number of steps and have involved the addition of either a very large amount of 35 basic refractory material such as lime or such a small amount of the basic refractory material, as to not attain a particularly high yield of the chromate, also a step of leaching, involving subsequent filtration, weighing, mixing and drying, preliminary to a retreatment 40 of the partly treated ore, all of which have involved great expense which I find unnecessary and undesirable.

Further objects of my invention will appear from the detailed description of the same hereinafter.

While my invention is capable of embodiment in many different forms, I have described hereinafter only certain forms of my 50 invention, by way of example, and while it is

of the air in proximity to the spray nozzle 12 in order to provide oxygen for the combustion of the fuel within the kiln. The burner 12 and pipe 13 are supported within a kiln 5 hood 13b, having angle adjusting screw supports 13c. These are supported from adjustable screw sleeves 13d carried by turnbuckles 13e from rollers 13f movable on a cross beam 13g supported on any suitable uprights 13h and 13i longitudinally adjustable on tracks 13j and 13k.

The resultant material escapes from the lower end of the rotary kiln 1 preferably in advance of the end of the shield pipe 13. 15 However, due to the upward flow of the burning fuel and the incoming air there is also a current of air entering the lower end of the kiln 1 and passing upwardly through the same outside of the shield tube 13. This arrangement is such as to provide a cooling zone for the downwardly moving materials around the tube 11 and pipe 13 in which the incoming air not only cools the materials passing downwardly therein, but also becomes heated, thereby assisting in the oxidation of the said materials throughout the kiln 1.

In carrying out my invention, for example, I might introduce into the kiln 1 through the hopper 9 a mixture of finely ground chrome ore containing, for instance:

100 parts by weight chrome ore (containing 50%  $\text{Cr}_2\text{O}_3$ )

70 parts by weight of lime

49 parts by weight of soda ash

In this mixture the lime may, however, vary from 70 parts to 80 parts by weight and, if desired, the soda ash may vary from 45 parts to 53 parts by weight. Also, the lime 30 may be any other basic refractory material and the soda ash may be substituted with any other alkali carbonate. It will be understood, also, that in this application wherever I refer to lime or soda ash such substitute materials 35 may be used if desired. This amount of basic refractory material is at least such as not only to prevent the formation of any undesirable compounds from the soda ash and the silica and alumina which is contained in the chrome ore, but is sufficient also to attain the high 40 yields of chromates hereinafter referred to. Also, the soda ash is present in sufficient quantity to combine with somewhat less than, that is to say, about 70% by weight of the chromic oxide present. This mixture is roasted in 45 the kiln at a temperature of about 1000° C., in the oxidizing atmosphere present therein in the upper part of the kiln, that is to say, between the upper end of the burner 12 and the upper end of the kiln, after which 50 the materials pass downwardly into the cooling zone, that is to say, between the upper end of the burner and the lower end of the kiln in which the average temperature is approx- 55 imately 800° C., so that the materials pass

out the lower end of the kiln at a temperature of about 600° C. The reactions which take place in the kiln 1 are as follows:



The treatment in the kiln 1 requires approximately 3 hours. 75

These materials delivered from the kiln 1 are in the form of particles varying in size from a fine powder to lumps 1 inch in diameter, the latter having been oxidized practically only at the surface thereof, and containing calcium chromate, sodium chromate as well as the silicates of lime and alumina. 80

These materials may be then subjected to a leaching operation in water, containing un- 85 combined sodium carbonate to decompose calcium chromate so as to form sodium chromate therefrom for a period of 24 hours, and is then filtered through any desired apparatus, the liquid which contains sodium chromate 90 being then evaporated or treated in any desired manner for the recovery of sodium chromate or sodium bichromate therefrom, according to the usual procedure. The leaching operation is preferably conducted at a 95 temperature of 80° C., and requires a period generally of 12 hours. The residue thus recovered from the filter is ground either wet or dry while mixed with enough soda ash which is added thereto in an amount either 100 to combine with somewhat less than the total chromic oxide present therein, that is to say, to combine with about 90% by weight of the chromic oxide present, or more up to an amount equal to about 110% of the theoretical 105 soda ash required to combine therewith. For example, this mixture may comprise 100 parts by weight of the dry residue (containing approximately 12% by weight  $\text{Cr}_2\text{O}_3$ ) and 15 parts by weight of soda ash, although the 110 soda ash may vary from 12 parts to 20 parts by weight of said residue. This mixture is then re-roasted in substantially the same way and under the same conditions as the first 115 roasting operation in the kiln 1. The materials thus obtained from the re-roasting may then be subjected also to leaching, filtration and evaporation in substantially the same way as described above after the first roasting. By this means I am enabled to obtain 120 a very high yield of the alkali chromate, inasmuch as a recovery corresponding to from 90% to 95% by weight of the chromic oxide present in the original chrome ore is recovered in the form of the alkali chromate or 125 bichromate, about  $\frac{3}{4}$  of this amount having been recovered from the first leaching following the first roasting operation.

If desired, however, I may conduct the 130 process in such a manner as to enable a very

much lower cost of production to be attained and in a much shorter interval of time, as follows:

In this modification of my invention the

5 process may be carried out in a manner somewhat similar to the form of my invention described in detail above. However, in this instance I prefer to mix together—

10 100 parts by weight of chrome ore (containing about 50% by weight of  $\text{Cr}_2\text{O}_3$ )  
80 parts by weight of lime  
63 parts by weight of soda ash.

Here, if desired, the lime or other basic refractory material may vary from 70 parts to 85 parts by weight and the soda ash or other alkali carbonate may vary from 60 parts to 66 parts by weight of the chrome ore. Here it will be noted that the amount of soda ash 15 present is sufficient to combine with about 90% by weight of the total chromic oxide present in the ore. This mixture is then passed through the kiln 1 under the same conditions of operation until the oxidation 20 of the chromic oxide is from 60% to 70% by weight completed. At this stage of the process no leaching operation is necessary. Instead, preferably, the materials thus treated, the same being in the form of a fine powder 25 up to lumps 1 inch in size, are ground to a fine powder and then run again through the kiln 1 under substantially the same conditions of operation and without the necessity of adding any further lime or soda ash there- 30 to. The materials thus treated are then subjected to a leaching operation under the same conditions of treatment referred to in the first leaching hereinabove described in connection 35 with the first embodiment of my invention, 40 after which the filtrate is evaporated to obtain sodium chromate, or bichromate and the residue may then be discarded. The yield of sodium chromate or bichromate thus obtained corresponds to a recovery of from 88% 45 to 92% by weight of the chromic oxide present in the chrome ore treated.

While I have described my invention above in detail it is to be understood that many changes may be made therein without departing from the spirit of my invention as 50 set forth in the claims.

I claim:

1. The process which comprises roasting chrome ore with a basic refractory material 55 and an alkali carbonate then grinding the product, re-roasting the said unleached product and recovering the alkali chromate therefrom.

2. The process which comprises roasting chrome ore with a basic refractory material 60 and an alkali carbonate, then grinding the product, re-roasting the said unleached product and recovering the alkali chromate therefrom by leaching, filtration and evaporation.

65 3. The process which comprises roasting

chrome ore with a basic refractory material and an alkali carbonate, re-roasting the said unleached product and recovering the alkali chromate therefrom.

4. The process which comprises roasting 70 chrome ore with a basic refractory material and an alkali carbonate, re-roasting the said unleached product and recovering the alkali chromate therefrom by leaching, filtration and evaporation. 75

JOSEPH J. VETTER.

80

85

90

95

100

105

110

115

120

125

130